

## UNITED STATES PATENT OFFICE

1,994,608

## MANUFACTURE OF ESTERS OF POLYMERIZED CARBOHYDRATES

Max Hagedorn, Dessau in Anhalt, Germany, assignor to I. G. Farbenindustrie Aktiengesellschaft, Frankfort-on-the-Main, Germany, a corporation of Germany

No Drawing. Application February 6, 1929, Serial No. 338,051. In Germany February 10, 1928

10 Claims. (Cl. 260—101)

My present invention relates to the manufacture of esters of polymerized carbohydrates and more particularly to an improvement in the known process of preparing such esters by acting with a chloride of organic acids of higher molecular weight upon polymerized carbohydrates treated with a caustic alkali with the effect of obtaining directly esters soluble in halogenated hydrocarbons. Another advantage of my invention is that the new products obtainable by this process are in a pure, nearly colorless state.

The esterification of polymerized carbohydrates with higher fatty acids has not hitherto been achieved without preliminary treatment, because of the incapacity of these carbohydrates to react on account of their colloidal character. It is only possible to esterify polymerized carbohydrates with higher fatty acids by previously causing them to swell in strong aqueous alkali hydroxide solutions. This treatment produces the known alkali compounds of the carbohydrates which, in a condition moist with water, can react with fatty acid halides.

For swelling the carbohydrates strong alkali hydroxides containing 30 per cent. and more of alkali hydroxide are necessary, since only in this case alkali compounds of the carbohydrates are formed which react easily. Such treatment leads, in the case of cellulose, to the compound  $(C_6H_{10}O_5)_2NaOH$ .

When the alkali compounds of the carbohydrates, as has been proposed for alkali cellulose, are esterified with acid halide in the usual manner, that is to say, accompanied by cooling, there are obtained insoluble esters which must be submitted to a separate and special treatment, since they acquire properties of solubility only by such further treatment.

According to the present invention esters which are soluble in organic agents are obtained in a single operation, when the operation is conducted without removing the heat of reaction evolved during the esterification. The reaction may be carried out with the addition of some more heat.

For the esterification of any polymerized carbohydrate the halide of an acid of a higher molecular weight may be used, that is to say, for instance of any saturated or unsaturated, substituted or unsubstituted fatty acid containing more than five carbon atoms or of an analogous cyclic carboxylic acid.

The esterification may be executed by the aid of a mixture of a fatty acid halide with another organic or inorganic acid halide, mixed esters thus being formed. For instance, there may be em-

ployed jointly a higher fatty acid halide, for example stearyl chloride or lauryl chloride, and any other acid halide, for example the chloride of acetic acid, benzoic acid, naphthenic acid.

While the known processes for making cellulose esters of higher fatty acids always lead to more or less strongly colored products, the products obtainable according to the present invention are quite colorless. These products are suitable for all the purposes for which hitherto carbohydrate derivatives have been suggested. They are particularly useful for making threads, films, lacquers, masses which can be spread with a knife, coatings on paper or fabric, insulating masses, plastic masses or the like. They may be moulded by pressure at a raised temperature below their melting point or may be used when dissolved in an organic solvent.

The new esters of polymerized carbohydrates derived from cyclic carboxylic acids, for example cyclopentane-carboxylic acid and cyclohexane-carboxylic acid, are colorless and dissolve completely in aromatic hydrocarbons, in chlorinated hydrocarbons and in fatty acid esters. In ether and in aliphatic hydrocarbons they swell strongly. These solubilities vary, if, besides the radicle of the cyclic carboxylic acid, still other acid radicles are introduced, and, furthermore, the solubilities vary according to the changes in the ratios, and with the nature of the said other radicles introduced.

The carbohydrate compounds which contain radicles of cyclohexane-carboxylic acids (naphthenic acids) exhibit the remarkable property that at ordinary temperature they are very hard and strong, while at moderate temperatures (about 50° C. and therefore far below their melting point, which is about 200° C.), they soften and are capable of being moulded. This property makes it possible to work them up without addition of a solvent or softening agent.

The following examples illustrate the invention:

Example 1.—10 grams of finely powdered rice starch are stirred quickly with 10 cc. of aqueous sodium hydroxide solution of 40 per cent. strength. The alkali starch thus obtained is suspended in 50 cc. of benzene and a mixture of 16 cc. of benzoyl chloride and 14 cc. of lauryl chloride is added. The heat of the reaction, which is soon developed, brings the benzene to gentle ebullition. The mixture is viscid throughout and finally solidifies to a jelly. From the latter, the sodium chloride, produced by the reaction, is washed out by means of water. The

5

10

15

15

20

25

30

35

40

45

50

55

residue insoluble in water consists, after thorough extraction with methanol, of pure, quite colorless starch-laurate-benzoate, which dissolves in dichloro-methane and swells strongly in benzene. Solutions of it may easily be filtered off from a small quantity of undissolved particles.

Example 2.—10 grams of cellulose are treated for 4 hours with an aqueous sodium hydroxide solution of 40 per cent. strength at  $-10^{\circ}$  C., to cause swelling and are then freed from an excess of alkali lye by pressing until the mass weighs 30 grams. The alkali-cellulose is suspended in 80 cc. of chloro-benzene. There are then added 80 cc. of lauryl chloride; the temperature of the mixture rises within 5 minutes from  $20^{\circ}$  C. to  $75$ – $80^{\circ}$  C. This temperature is maintained for about 15 minutes. There is produced a cloudy, viscid solution which, after about 30 minutes solidifies to a jelly. This mass is extracted several times with boiling alcohol and water and then dried. 23 grams of a snow white cellulose laurate soluble in benzene and in dichloro-methane are obtained.

Example 3.—10 grams of agar-agar, in the form of a powder fine as dust, are stirred with 10 cc. of aqueous caustic soda solution of 40 per cent. strength. Swelling is allowed to continue for 15 minutes, and the mass is then dispersed by strongly shaking in 50 cc. of benzene. On addition of 50 cc. of a mixture of the chlorides of cocoanut oil fatty acids, the suspension is converted, with strong evolution of heat, into a thickish jelly. The carbohydrate derivative is precipitated with ethanol and extracted by boiling water to free it from the salts soluble in water and fatty acids, which have been formed by the reaction. There is thus obtained a cocoanut oil fatty acid ester of that carbohydrate of agar-agar, which forms the fundamental constituents thereof; the product is snow white, clearly soluble in aromatic and in chlorinated aliphatic hydrocarbons.

Example 4.—10 grams of cellulose are softened for 3 hours at  $-12^{\circ}$  C. in an aqueous sodium hydroxide solution of 40 per cent. strength and the alkali cellulose thus produced is freed from the excess of lye by pressing to a weight of 30 grams. The alkali cellulose, composed of 10 grams of cellulose, 8 grams of caustic soda and 12 grams of water, is comminuted and suspended in 80 cc. of chlorobenzene. There is then added a mixture of 60 cc. of naphthenic acid chloride (boiling point  $95$ – $135^{\circ}$  C. at 12 mm. pressure) and 20 cc. of pure distilled lauryl chloride, whereby the mixture becomes heated to about  $85^{\circ}$  C. and milky and thick. The course of the reaction is accelerated by warming on the steam-bath. The reaction is finished after about 1 hour. By precipitation with alcohol and extraction with boiling alcohol and water there is isolated a white cellulose naphthenate-laurate, which is soluble in aromatic and in chlorinated aliphatic hydrocarbons. It may be pressed to thin, transparent colorless plates by the process described in application Serial Number 269,294 filed April 11, 1928.

Example 5.—10 grams of starch are stirred with a solution of 12 grams of sodium hydroxide in 18 grams of water until a homogeneous gelatinous mass has been produced. This mass is introduced slowly into a mixture of 47 grams of phenyl-acetic acid chloride and 60 cc. of benzene. The heat of reaction evolved heats the mixture up to the boiling point of the benzene. The mixture is allowed to stand for 24 hours, and then

4 times its weight of methanol are added; the ester separates from the liquid and is washed four times with methanol and then thoroughly with hot water. This ester contains 70 per cent. of bound phenyl-acetic acid and dissolves in halogenated hydrocarbons.

As can be seen from the foregoing examples, I may introduce into the molecule of the polymerized carbohydrate either an aliphatic acid with more than five carbon atoms or a cyclic carboxylic acid with more than five carbon atoms or a mixture of these compounds. In the following claims the term "organic acid with more than five carbon atoms" is intended to include aliphatic as well as cyclic carboxylic acids.

I claim:

1. The process of manufacturing cellulose naphthenate laurate which comprises swelling cellulose in an aqueous alkali metal hydroxide solution of at least 30 per cent. strength, acting upon the wet alkali metal cellulose simultaneously with lauric acid chloride and naphthenic acid chloride and promoting the reaction by the heat formed in this esterification process.

2. Cellulose naphthenate laurate soluble in aromatic and in chlorinated aliphatic hydrocarbons, being of white appearance and forming when pressed transparent colorless plates.

3. The process of manufacturing starch-laurate-benzoate which comprises producing alkali starch by mixing finely powdered rice starch with an aqueous solution of sodium hydroxide of 40 per cent strength, suspending the alkali starch in a mixture of benzoyl chloride and lauryl chloride in benzene, and promoting the reaction by the heat formed in this esterifying process.

4. The process of manufacturing the cocoanut oil fatty acid ester of agar-agar which comprises mixing finely powdered agar-agar with an aqueous solution of sodium hydroxide of 40 per cent strength, dispersing the reaction mass by strongly shaking with benzene, adding a mixture of the chlorides of cocoanut oil fatty acids, and promoting the reaction by the heat formed in this esterifying process.

5. The process of manufacturing an ester of a polymerized carbohydrate which comprises swelling the polymerized carbohydrate in an aqueous solution of an alkali metal hydroxide of at least 30 per cent strength to form an alkali metal compound, finely distributing said alkali metal compound in a solvent for said ester, and acting on said alkali metal compound with a mixture of halides of acids, selected from the group consisting of aliphatic acids with more than 5 carbon atoms and of benzoic acid without removal of the heat of reaction formed in the said esterifying process.

6. The process of manufacturing a cellulose ester which comprises swelling cellulose in an aqueous solution of an alkali metal hydroxide of at least 30 per cent strength to form alkali cellulose, finely distributing said alkali cellulose in a solvent for said cellulose ester and acting on said alkali metal compound with a mixture of halides of acids, selected from the group consisting of aliphatic acids with more than 5 carbon atoms and of benzoic acid without removal of the heat of reaction formed in the said esterifying process.

7. The process of manufacturing an ester of a polymeric carbohydrate which comprises swelling the polymeric carbohydrate in an aqueous solution of an alkali metal hydroxide of at least 30 per cent strength to form an alkali metal com-

pound, finely distributing said alkali metal compound in a solvent for said ester, and acting on said alkali metal compound with a halide of a higher fatty acid with more than five carbon atoms and with a halide of naphthenic acid.

5. The process of manufacturing a cellulose ester which comprises swelling cellulose in an aqueous solution of an alkali metal hydroxide of at least 30 per cent strength to form alkali cellulose, finely distributing said alkali cellulose in a solvent for said cellulose ester, and acting on said alkali cellulose with a halide of a higher fatty acid with more than five carbon atoms and with a halide of naphthenic acid.

10. The process of manufacturing cellulose laurate naphthenate which comprises producing alkali cellulose by mixing cellulose with an aqueous

solution of sodium hydroxide of 40 per cent strength at  $-12^{\circ}$  C., suspending the alkali cellulose in chlorobenzene, adding naphthenic acid chloride and lauryl chloride in the ratio 6:2 parts by volume and promoting the reaction by the heat formed in this esterifying process.

15. The process of manufacturing cellulose laurate which comprises producing alkali cellulose by mixing cellulose with an aqueous solution of sodium hydroxide of 40 per cent strength at  $-10^{\circ}$  C., pressing the alkali cellulose formed to three times its original weight, suspending the alkali cellulose in chlorobenzene, adding lauryl chloride, and promoting the reaction by the heat formed in this esterifying process.

MAX HAGEDORN.